

# UNITED STATES PATENT OFFICE.

ERNST MARMETSCHKE, OF SCHÖPFURTH, NEAR EBERSWALDE, GERMANY, ASSIGNOR  
TO HUBERTUSMÜHLE MIT BESCHRÄNKTER HAFTUNG, OF SCHÖPFURTH, GERMANY.

## PROCESS OF PRESERVING WOOD.

1,016,024.

Specification of Letters Patent.

Patented Jan. 30, 1912.

No Drawing.

Application filed December 10, 1910. Serial No. 596,712.

To all whom it may concern.

Be it known that I, ERNST MARMETSCHKE, subject of the Emperor of Germany, residing at Schöpfurth, near Eberswalde, 5 Prussia, Germany, have invented certain new and useful Improvements in Processes of Preserving Wood, of which the following is a specification.

In Letters Patent of the United States 10 #898,246, granted September 8, 1908, I have described a process in which the wood to be treated is subjected to the action of a preservative solution composed of zinc chlorid and aluminium sulfate, at an effective 15 low temperature of 60° C., the highest temperature not to exceed 98° C. About 60° C., or between 60° C. and 65° C. coagulation of the colloidal constituents takes place, and if the temperature does not reach 20 60° it is ineffective to establish permanent impregnation and hence the minimum temperature stated in my former patent.

I have now discovered that the process 25 of my former patent can be carried out with greater effectiveness by first subjecting the wood to be treated to the action of the preservative solution at a temperature below that where the fixing of the salts take place, so as to allow the wood to become 30 thoroughly saturated and absorb the greatest quantity of the preservative material. Thereafter the wood in the immediate presence of the injected salts is heated to a temperature sufficient to coagulate the 35 colloidal constituents. This has the effect of closing the wood cells and permanently incasing the preservative therein.

To carry out the process I use a storage 40 tank for storing and heating the solution, a pressure cylinder with fittings, vacuum, and pressure pumps as in the known processes for impregnating timber, with connections for blowing live steam into the cylinder. I make up the solution preferably 45 with a 3% solution of zinc chlorid and a 1.5% solution of aluminium sulfate and after subjecting the timber in the pressure cylinder to a vacuum, draw in the solution at a temperature of about 55° centigrade.

I then force this solution into the timber 50 under pressure. When sufficient of the preservative solution has been injected I release the pressure and raise the temperature of the timber, still immersed in the solution, to about 70° centigrade and keep 55 it at this temperature, for about an hour. This temperature and time are sufficient to secure coagulation of the colloidal constituents and permanent incasing of the preservative in the cells of the wood, so that it 60 cannot be washed out.

If the solution is injected below the coagulating point of the colloidal constituents and the timber not subsequently heated above 60° centigrade the salts are easily 65 lixiviated and if the whole process is carried out above 60° centigrade the colloidal constituents coagulate before the injection is complete so that the amount which can be injected is limited and the salts cannot 70 be incased or combined by further heating.

The invention is not to be confined to the exact temperatures above stated as the essential feature consists in the injection of the preservative solution at a temperature below that at which the colloidal constituents 75 coagulate, while the material is subsequently heated above this point. Similarly any equivalents of the salts specified may be employed.

What I claim is:—

1. A process of preserving wood and other fibrous materials which consists in first injecting a preservative solution into the material at a temperature below that at 85 which the colloidal substances contained therein coagulate and subsequently raising the temperature of the wood above this temperature for the purpose set forth.

2. A process of preserving wood and 90 other fibrous materials which consists in forcing a solution of zinc chlorid and aluminium sulfate at a temperature of about 55° C. into the material and subsequently raising the temperature of the material to 95 about 70° C. substantially as and for the purpose hereinbefore set forth.

3. A process of preserving wood and the

like consisting in subjecting the wood or other material to a vacuum, in a closed vessel, introducing into said vessel an impregnating solution consisting of zinc chloride and aluminium sulfate at a temperature

raising the temperature above the coagulating point, substantially as described. 10

In testimony whereof, I affix my signature in presence of two witnesses.

ERNST MARMETSCHKE.

Witnesses:

KUNO SCHAEFFER,

CURT MÜLLER.